

May 31, 1927.

1,630,715

B. G. NICE

METHOD OF MAKING BALL CONE ELEMENTS

Filed Jan. 18, 1923



FIG. 1.



FIG. 2.



FIG. 3.



FIG. 4.



FIG. 5.



FIG. 6.

WITNESS:

Robt R. Kitchel.

Budd G. Nice  
BY  
Augustus R. Strongton  
ATTORNEY

Patented May 31, 1927.

1,630,715

# UNITED STATES PATENT OFFICE.

BUDD G. NICE, OF OGONTZ, PENNSYLVANIA, ASSIGNOR TO ARTHUR N. GOODFELLOW,  
OF PHILADELPHIA, PENNSYLVANIA, TRUSTEE.

## METHOD OF MAKING BALL-CONE ELEMENTS.

Application filed January 18, 1923. Serial No. 613,489.

The product of the method of this invention is a ball-cone element consisting of a body portion of flaring tubular form provided at its flaring end with a flat flange 5 and at its other end with a cylindrical flange right-angularly disposed in respect to the flat flange.

The principal object of the present invention is to provide a simple, expeditious and 10 comparatively inexpensive method of making such ball-cone elements from sheet metal stock and, generally stated, the method consists in producing from such stock metal blanks of flat ring form and then enlarging 15 the hole in the blank and drawing and stretching and bending the metal adjacent to the hole in respect to the flat metal remote from the hole and disposed at the outer rim of the blank by the application of pressure 20 to the face of the blank.

The invention also comprises the improvements to be presently described and finally claimed.

In the description reference will be made 25 to the accompanying drawing forming part hereof and in which

Figure 1 is a cross-sectional view of a ball bearing fitted with a ball-cone element which is the product of the method of the present 30 invention.

Fig. 2 is an elevational view of the ball-cone element.

Fig. 3 is a top or plan view illustrative of 35 the manufacture of the metal blanks of flat ring form from sheet metal stock.

Fig. 4 is an elevational view, principally in cross-section, further illustrative of the manufacture of the flat ring blanks, and

Figs. 5 and 6 are elevational views, principally in cross-section, illustrating the manufacture of a ring blank into a ball-cone by the method of the present invention.

The ball-cone consists of a body portion 1 of tubular flaring form provided at its flaring end with a flat flange 2 and at its other end with a cylindrical flange 3 disposed right-angularly in respect to the flange 2. A sheet of flat metal 4 of appropriate thickness and width is the stock from which metal 50 blanks of flat ring form 5, Fig. 5, are produced. One way of doing this is to feed the stock or sheet 4 from right to left through a punch and die mechanism of which parts are indicated in Fig. 4. The piercing punch 55 6 in co-operation with the die 7 removes a

circular slug from the sheet 4 and the opening thus formed is the hole 8 at the center of the blank of ring form and is also useful in co-operating with the pilot pin 9 of the punch 10 for the production of the ring 60 blank. It may be said that the knock-out and guide mechanisms are omitted from Fig. 4 because they are too well understood by those skilled in the art to require illustration. The hole 8 in the blank of flat ring 65 form 5 is enlarged and the metal adjacent to the hole 8 is drawn, stretched, bent and displaced laterally in respect to the flat metal remote from the rim of the hole, thus producing the ball-cone element already 70 described. Referring to Figs. 5 and 6 for a further description of the method of the invention, the blank of flat ring form is supported at its outer margin 2 on the rim of a flaring opening in the die 11, and the blunt point 12 of the forming punch 13 enters the hole 8 and the flat end of the body of the punch 13 applies pressure to the flat face of the blank and forces the center of the blank 75 downward, draws the metal around the curved surface of the opening in the die, and forces the hole open, stretching the metal, and bends the center edge of the blank into the flange 3. The metal of the blank surrounding the hole flows ahead of the end of the body of the punch. Finishing the downward stroke the punch holder 14 strikes the top surface of the spring retracted flattening punch 15 and causes it to 80 strike the top surface of the blank and flatten 85 it to size. On the up-stroke the part 15 strips the finished product from the part 13. The product of the method may be placed 90 in a revolving gas carburizing furnace and gradually brought to the necessary temperature for case hardening. The heated product can then be removed and quenched in water and thereafter sand-blasted to remove surface scale formed during the heat treatment. Of course other means than a revolving gas carburizing furnace may be employed for heating the product. 100

From the foregoing description and upon reference to the drawings it is evident that the blank is unconfined at the outer part when the pressure makes the tubular part, and that the tubular part is confined when the continued pressure is applied to the outer rim to flatten it, as in Fig. 6.

It will be obvious to those skilled in the art 110

to which the invention relates that modifications may be made in details of procedure and in matters of mere form without departing from the spirit of the invention which 5 is not limited in respect to such considerations or otherwise than as the prior art and the appended claim may require.

I claim:

10 The method of making ball-cone elements in two stages and at one operation from metal blanks of flat ring form which consists in flaring the inner rim parts of the blank

laterally out of the plane of the outer rim parts and into flaring tubular and cylindrical form by pressure applied to the portion 15 of the face of the blank which lies between the rim of the hole and the margin of the blank while the outer part of the blank is unconfined, and then flattening the previously unconfined outer rim portion of the 20 blank by continued pressure applied in the same direction while the flaring tubular part is confined.

BUDD G. NICE.